

E. BENEDICTUS,  
MANUFACTURE OF STRENGTHENED GLASS,  
APPLICATION FILED JUNE 14, 1911.  
1,182,739.

Patented May 9, 1916.

Fig. 1



Fig. 2



WITNESSES  
L. H. Grote  
W. G. Keir

INVENTOR

EDOUARD BENEDICTUS  
By Harmanus Harman  
his Attorneys

# UNITED STATES PATENT OFFICE.

EDOUARD BENEDICTUS, OF PARIS, FRANCE.

## MANUFACTURE OF STRENGTHENED GLASS.

1,182,739.

Specification of Letters Patent.

Patented May 9, 1916.

Application filed June 14, 1911. Serial No. 633,128.

*To all whom it may concern:*

Be it known that I, EDOUARD BENEDICTUS, of 25 Rue de Fourcroy, Paris, France, artistic painter, have invented certain new 5 and useful Improvements in the Manufacture of Strengthened Glass, of which the following is a full, clear, and exact description.

This invention relates to a new process 10 for the manufacture of the strengthened glass which forms the subject of my application for Letters Patent filed January 11th, 1910, Serial No. 537,557, and my application for Letters Patent filed June 13, 1911, Serial No. 632,850.

This process relates more particularly to the case of a strengthening layer composed wholly or in part of gelatin. Gelatin, which liquefies at a comparatively low temperature, presents the advantage of being readily attachable to glass or celluloid under the action of moderate heat completed if necessary by the application of pressure and without requiring the use of a solvent to 25 soften the surfaces which are to be stuck together. Nevertheless gelatin is a hygroscopic substance which in spite of attempted drying may easily retain moisture which prejudicially affects the solidity and the 30 transparency of the finished strengthened glass.

The present invention consists in subjecting the gelatin at the moment of sticking, to a liquid which is both hygroscopic 35 and volatile, in such a way as to dehydrate the gelatin and then to remove by evaporation at the same time as the water the air which remained therein during the sticking. Moreover, it is advantageous to employ for 40 this purpose a liquid which is inert to gelatin, that is neither dissolving nor attacking that substance, so that it may be expelled rapidly under the action of heat which is not the case when a solvent which incorporates itself therein is used to soften the 45 surface of the gelatin; in the latter case the last traces of the solvent are difficult to eliminate.

The liquid employed is preferably ethyl 50 alcohol of 95%, denatured or not. If denatured alcohol is used for economy, methylic denaturation is the method to be preferred. The figure of 95% above given is only by way of example, but it is advisable not to

lower the strength below 75%, because there 55 would then be produced a fog caused by moisture in the gelatin.

The following example describes a method of making strengthened glass according to this invention: In the first place 60 the face of the glass plates which is to contact with the gelatin is cleaned as thoroughly as possible; this is important to insure the perfect adhesion of the gelatin upon the glass. The cleaning may be effected by using rouge or tripoli in suspension in water; the glass is then rinsed and dried without being touched. Other methods of cleaning may of course be employed. The glass plates are then dipped 70 in a bath of ethyl alcohol and applied on either side of the sheet of gelatin. The whole is then laid between the tables of a hydraulic or other press heated by steam or water circulation and a pressure of several kilograms (for example eight kilograms) per square centimeter is applied. The heat softens the gelatin and its action combined with that of the pressure effects 75 the sticking of the same to the glass, while 80 the liquid is expelled together with the moisture of the gelatin and the contained air.

In place of ordinary gelatin, there may be employed gelatin which is bleached and rendered supple and tenacious by incorporation of albumin, fibrin and protein or also nitrocellulose, as indicated in the specification of my application for Letters Patent filed June 13, 1911, Serial No. 632,850. 85

Instead of preparing the sheet of gelatin beforehand, the material may be poured upon one of the glass plates, the whole being then dipped in alcohol and the second glass plate applied under heat and pressure. 90

When the glass is to be strengthened by a layer of celluloid coated with gelatin, the latter is substituted for the gelatin sheet as indicated in the above mentioned specification, the method of attaching this strengthening layer between the glass plates being identical with that described in the case of gelatin alone. But in this case it is advantageous to adopt the following procedure: Upon each of the well-cleaned glass plates 105 there is poured an aqueous solution of gelatin, which is allowed to dry so as to obtain upon each plate a very thin adherent film

of gelatin. The two glass plates are dipped in alcohol and there is inserted between them (on the side of the gelatin film) a sheet of celluloid; the whole is then submitted to heat and pressure as above described. The alcohol in this way introduced between the gelatin and the celluloid exerts no appreciable solvent action upon the celluloid under the conditions of this 10 method of operation, but as above stated the alcohol dehydrates the gelatin and removes the air contained between the celluloid and the gelatinized faces of the glass.

To insure the preservation of the strengthened glass so made, and to prevent rehydration of the gelatin as well as any return of air between the gelatin and the glass along the periphery of the strengthened glass, the edges of the sheet may be luted. This luting may be effected for example by insolubilizing the periphery of the gelatin sheet by one or other of the following processes or any equivalent:—The strengthened glass is dipped for three hours in a saturated solution of bichromate of potash; the latter penetrates into the gelatin for an approximate distance of two millimeters and after exposure to sunlight it becomes insoluble and forms a sound joint. The glass is exposed for some days to vapors of formol which penetrate by diffusion for eight to ten millimeters and render the gelatin insoluble. Before inserting the gelatin between the glass plates, its edges are dipped 30 in a saturated solution of bichromate of potash and after the making of the strengthened glass it is exposed to sunlight; this luting is hermetic. Again the luting may be effected by applying paraffin, pitch 35 or the like along a marginal space afforded all along the periphery of the sheet of armored glass by the use of a layer of strengthening material of slightly smaller dimensions than the glass plates.

One or other of the above processes will be employed according to circumstances. For example the second process (by means of formol) will be applied to glass re-cut or retrimmed to size, while the others will be applied preferably to glass of definite dimensions, such as windows for carriages, conservatories, railways and the like.

In the accompanying drawing, Figure 1 is a section through reinforced glass in which the two glass sheets are united by a sheet of gelatin alone; Fig. 2 is a like view in which a sheet of celluloid is interposed between gelatin sheets on the adjacent faces of the two sheets of glass.

In these drawings *a* and *b* represent the sheets of glass between which is interposed a sheet of gelatin *c*, in Fig. 1, and two films of gelatin *c*<sup>1</sup> and *c*<sup>2</sup>, separated by a film of celluloid *d*, in the form shown in Fig. 2.

Having thus described my invention, what

I claim as such and desire to secure by Letters Patent is:—

1. The process of reinforcing glass, which consists in pressing a substance comprising gelatin between sheets of glass in the presence of heat and a volatile, hygroscopic liquid inert to gelatin, substantially as and for the purpose described. 70

2. The process of reinforcing glass, which consists in treating a substance comprising gelatin with a volatile, hygroscopic liquid inert to gelatin, and immediately pressing said substance between sheets of glass in the presence of heat. 75

3. The process of reinforcing glass, which 80 consists in treating a sheet comprising gelatin with ethyl alcohol almost free of water (alcohol approximately at 90-95%) and immediately pressing said sheet between sheets of glass in the presence of heat. 85

4. The process of reinforcing glass, which consists in subjecting a sheet of reinforcing material comprising gelatin to the action of a volatile, hygroscopic liquid inert to gelatin and at once compressing said sheet between sheets of glass in the presence of heat. 90

5. The process of reinforcing glass, which 95 consists in subjecting a sheet of reinforcing material comprising gelatin to the action of a volatile, hygroscopic liquid inert to gelatin and at once compressing said sheet between sheets of glass in the presence of heat, and thereafter luting the edges of the article thus produced to prevent the rehydration of the gelatin, substantially as described. 100

6. The process of reinforcing glass which 105 consists in subjecting to pressure in the presence of heat a composite comprising a sheet of celluloid, a film of gelatin on each side thereof and sheets of glass outside the gelatin, the gelatin being subjected to the action of a volatile, hygroscopic liquid immediately in advance of said pressure, for the purpose described.

7. The process of reinforcing glass which 110 consists in subjecting to pressure in the presence of heat a composite comprising a sheet of celluloid, a film of gelatin on each side thereof and sheets of glass outside the gelatin, the gelatin being subjected to the action 115 of a volatile, hygroscopic liquid inert to gelatin immediately in advance of said pressure, for the purpose described.

8. The process of reinforcing glass which 120 consists in assembling a sheet of celluloid between two sheets of glass, each of the latter having on its juxtaposed face a film of gelatin, and subjecting said composite to pressure in the presence of heat and in the presence of a volatile hygroscopic liquid in 125 contact with the gelatin, for the purpose described.

9. The process of reinforcing glass which 130 consists in assembling a sheet of celluloid between two sheets of glass, each of the lat-

ter having on its juxtaposed face a film of gelatin, and subjecting said composite to pressure in the presence of heat and in the presence of a volatile hygroscopic liquid in contact with the gelatin and inert thereto, for the purpose described.

10. The process of reinforcing glass which consists in applying a solution of gelatin to the faces of glass sheets, permitting the solution to dry whereby a film of gelatin is formed on the faces of said sheets, dipping said sheets in a bath of volatile hygroscopic liquid, immediately assembling a sheet of celluloid between them adjacent the gelatin and subjecting the composite to pressure in the presence of heat.

15. The process of reinforcing glass which consists in applying a solution of gelatin to the faces of glass sheets, permitting the solution to dry, wherebv a film of gelatin is

formed on the faces of said sheets, dipping said sheets in a bath of volatile hygroscopic liquid inert to gelatin, immediately assembling a sheet of celluloid between them adjacent the gelatin and subjecting the composite 25 to pressure in the presence of heat.

12. As a new article of manufacture, a sheet of celluloid faced on both sides and in the order named by sheets of gelatin and glass, all rigidly and autogenously united together, and the gelatin being substantially free from contained moisture, as described.

10 In testimony whereof I have signed my name to this specification, in the presence of two subscribing witnesses.

EDOUARD BENEDICTUS.

Witnesses:

CHARLES DONY,  
LEON PEILLET